# EUROPEAN PATENT SPECIFICATION

(11) **EP 1 516 827 B1**
(45) Date of publication and mention of the grant of the patent: **25.07.2007**
(21) Application number: 04027190.0
(22) Date of filing: 15.05.2001
(51) Int. Cl.: B65D 81/24

(54) **Packaging of bananas**
Verpacken von Bananen
Emballage des bananes

(30) Priority: 26.05.2000 US 580379
(43) Date of publication of application: 23.03.2005
(62) Divisional of application: 01959756.6
(73) Proprietor: Apio, Inc., Guadelupe, CA 93434 (US)
(72) Inventor: Clarke, Raymond, Los Altos, CA 94024 (US)
(74) Representative: Hall, Robert Leonard

(56) References cited:
- EP-A- 0 311 423
- WO-A-00/04787
- WO-A-92/10414
- WO-A-96/38495
- US-A- 3 450 542
- US-A- 6 013 293

## Description

This invention relates to the packaging of bananas.

This application is a divisional of EPA 01959756.6, now EP 1289855, which claims methods of ripening green bananas which comprise placing a sealed package containing the bananas in an ethylene-containing atmosphere. The sealed container has an oxygen permeability at 13°C per kg of bananas (OP13/kg) of at least 700 ml/atm. 24 hrs, an R ratio at 13 °C of at least 2 and an ethylene permeability at 13 °C per kg of bananas (EtOP13/kg) which is at least 3 times the OP13/kg of the container. The container includes an atmosphere control member which comprises a gas-permeable membrane comprising a microporous polymeric film having a polymeric coating thereon.

Respiring biological materials consume oxygen (O₂) and produce carbon dioxide (CO₂) at rates which depend upon temperature and the stage of their development. Ideally, a respiring material should be stored in a container whose permeability to O₂ and CO₂ is correlated with (i) the atmosphere outside the package, (ii) the rates at which the material consumes O₂ and produces CO₂, and (iii) the temperature, to produce the desired atmosphere within the container. This is the principle behind the technology of controlled atmosphere packaging (CAP) and modified atmosphere packaging (MAP), as discussed, for example, in US Patent Nos. 3,450,542 (Badran), 3,450,544 (Badran et al.), 3,798,333 (Cummin et al. 4,734,324 (Hill), 4,830,863 (Jones), 4,842,875 (Anderson), 4,879,078 (Antoon), 4,910,032 (Antoon), 4,923,703 (Antoon), 5,045,331 (Antoon), 5,160,768 (Antoon), 5,254,354 (Stewart) and 6,013,293 (De Moor), International Publication Numbers WO 94/12040 (Fresh Western), WO 96/38495 (Landec) and WO 00/04787 (Landec), and European Patent Applications Nos. 0,351,115 and 0,351,116 (Courtaulds).

As discussed in EP 1289855, bananas are respiring biological materials whose storage and ripening present the serious problems.

The invention claimed in this divisional application mitigates or overcomes one or more of these problems by packaging bananas in a bag (or other container) having designed permeabilities to O₂, CO₂ and ethylene. This invention makes it possible to maintain bananas, before and/or after their climacteric, in a packaging atmosphere which enables storage and/or ripening of the bananas in a controlled fashion, for example so that bananas can be ripened while they are being transported (for example on a ship) so that the bananas are at a desired color stage when they reach their destination. Some embodiments of the invention also make it possible to store bananas, after their climacteric, within a desired range of color stages (e.g. within the range most attractive for retail sale) for a longer period than is possible under conventional practice.

In a first aspect, this invention provides a package which comprises
(a) a sealed container, the sealed container including at least one atmosphere control member which provides a pathway for O₂, CO₂ and ethylene to enter or leave the packaging atmosphere and which comprises a gas-permeable membrane comprising
   (a) a microporous polymeric film, and
   (b) a polymeric coating on the microporous film
   preferably an atmosphere control member as described in WO 00/04787, referred to above; and
(b) within the sealed container, bananas, for example green bananas, and a packaging atmosphere around the bananas;
the sealed container having an O₂ permeability at 13 °C, per kg of bananas in the container (OP13/kg), of at least 700, preferably at least 1000, particularly at least 1500, ml/atm.24 hrs, an R ratio at 13 °C of at least 2, preferably at least 3, and an ethylene permeability at 13 °C, per kg of bananas in the container (EtOP13/kg) which is at least 3 times, preferably at least 4 times, the OP13/kg of the container.

The package is preferably stored in air at a temperature of 13-21°C, e.g. 13-18°C or 16-21°C.

The packaging atmosphere contains oxygen and carbon dioxide, and also ethylene, the ethylene being derived from the bananas themselves, or from a ripening room, or from a source of ethylene placed within the container before the container is sealed around the bananas. The packaging atmosphere changes substantially during the ripening process, as the bananas consume oxygen and generate carbon dioxide. Preferably, the packaging atmosphere, for part of the period before the bananas reach their climacteric, contains at least 10% preferably at least 12%, particularly 14 to 19%, of O₂, and less than 10%, preferably less than 4%, of CO₂, with the total quantity of O₂ and CO₂ being less than 20 %, preferably less than 17 %. Preferably, for at least part of the period after the bananas have passed their climacteric, the packaging atmosphere contains at least 0.8%, preferably 1.5 to 6%, especially 1.5 to 3%, of O₂, and less than 15%, preferably less than 7%, of CO₂ , with the total quantity of O₂ and CO₂ being less than 16%, preferably less than 10 %.

In this specification, including the Examples and the Claims below, reference is made to particular features of the invention. It is to be understood that the disclosure of the invention in this specification includes all appropriate combinations of such particular features. For example where a particular feature is disclosed in the context of a particular aspect or embodiment of the invention, or a particular claim, that feature can also be used, to the extent appropriate, in the context of other particular aspects and embodiments of the invention, and in the invention generally.

In describing and claiming the invention below, the following abbreviations, definitions, and methods of measurement are used. OTR is O₂ permeability. COTR is CO₂ permeability. EtTR is ethylene transmission rate. OTR, COTR and EtTR values are given in ml/m².atm.24 hrs; in some cases, the equivalent in cc/100 inch².atm.24 hrs is given in parentheses. OTR and COTR values referred to herein can be measured using a permeability cell (supplied by Millipore) in which a mixture of O₂, CO₂ and helium is applied to the sample, using a pressure of 0.7 kg/cm² (10 psi) except where otherwise noted, and the gases passing through the sample were analyzed for O₂ and CO₂ by a gas chromatograph. The cell could be placed in a water bath to control the temperature. The abbreviation P₁₀ is used to denote the ratio of the oxygen permeability at a first temperature T₁°C to the oxygen permeability at a second temperature T₂, where T₂ is (T₁-10)°C, T₁ being 10°C and T₂ being 0°C unless otherwise noted. The abbreviation R or R ratio is used to denote the ratio of C0₂ permeability to O₂ permeability, both permeabilities being measured at 20°C unless otherwise noted. Pore sizes given in this specification are measured by mercury porosimetry or an equivalent procedure. Parts and percentages are by weight, except for percentages of gases, which are by volume; temperatures are in degrees Centigrade, and molecular weights are weight average molecular weights expressed in Daltons. For crystalline polymers, the abbreviation Tₒ is used to denote the onset of melting, the abbreviation Tₚ is used to denote the crystalline melting point, and the abbreviation ΔH is used to denote the heat of fusion. Tₒ, Tₚ and ΔH are measured by means of a differential scanning calorimeter (DSC) at a rate of 10°C/minute and on the second heating cycle. Tₒ and Tₚ are measured in the conventional way well known to those skilled in the art. Thus Tₚ is the temperature at the peak of the DSC curve, and Tₒ is the temperature at the intersection of the baseline of the DSC peak and the onset line, the onset line being defined as the tangent to the steepest part of the DSC curve below Tₚ.

Where reference is made herein to sealing bags containing bananas, it is to be understood that the sealing can be, but generally is not, hermetic sealing. Conventional methods for sealing bags of bananas can conveniently be used in this invention. Such conventional methods include, for example, the use of a cable tie to seal the neck of the bag. A seal made by conventional methods is not a hermetic seal, and has the advantage that it permits equilibration of the pressures inside and outside the bag. If the bag is sealed hermetically, it will generally be desirable to include one or more pinholes in the bag, to achieve such equilibration.

As noted above, this invention makes use of an atmosphere control member comprising (a) a microporous polymeric film, and (b) a polymeric coating on the microporous film. The microporous polymeric film preferably comprises a network of interconnected pores having an average pore size of less than 0.24 micron, with at least 70% of the pores having a pore size of less than 0.24 micron. Preferably the pores in the microporous film constitute 35 to 80% by volume of the microporous film. Preferred microporous films comprise a polymeric matrix comprising (i) an essentially linear ultrahigh molecular weight polyethylene having an intrinsic viscosity of at least 18 deciliters/g, or (ii) an essentially linear ultrahigh molecular weight polypropylene having an intrinsic viscosity of at least 6 deciliters/g, or (iii) a mixture of (i) and (ii). The microporous film may contain 30 to 90% by weight, based on the weight of the film, of a finely divided particulate substantially insoluble filler which is distributed throughout the film. A preferred process for preparing suitable microporous films comprises
(A) preparing a uniform mixture comprising the polymeric matrix material in the form of a powder, the filler, and a processing oil;
(B) extruding the mixture as a continuous sheet;
(C) forwarding the continuous sheet, without drawing, to a pair of heated calender rolls;
(D) passing the continuous sheet through the calender rolls to form a sheet of lesser thickness;
(E) passing the sheet from step (D) to a first extraction zone in which the processing oil is substantially removed by extraction with an organic extraction liquid which is a good solvent for the processing oil, a poor solvent for the polymeric matrix material, and more volatile than the processing oil;
(F) passing the sheet from step (E) to a second extraction zone in which the organic extraction liquid is substantially removed by steam or water or both; and
(G) passing the sheet from step (F) through a forced air dryer to remove residual water and organic extraction liquid.

The polymeric coating on the control member preferably comprises a crystalline polymer having a peak melting temperature Tp of -5 to 40 °C, e.g. 0 to 15°C, or 10 to 20 °C, an onset of melting temperature Tₒ such that (Tₚ- Tₒ) is less than 10 °C, and a heat of fusion of at least 5 J/g. The polymer preferably comprises a side chain crystalline polymer moiety comprising, and optionally consisting of, units derived from (i) at least one n-alkyl acrylate or methacrylate (or equivalent monomer, for example an amide) in which the n-alkyl group contains at least 12, preferably at least 14, for example 16-50, preferably 16-22, carbon atoms, for example in amount 35-100%, preferably 50-100%, often 80-100%, and (ii) one or more comonomers selected from acrylic acid, methacrylic acid, and esters of acrylic or methacrylic acid in which the esterifying group contains less than 10 carbon atoms. The polymer can be a block copolymer in which one of blocks is a crystalline polymer as defined and the other block(s) is crystalline or amorphous. Preferred block copolymers comprise polysiloxane polymeric blocks, and (ii) crystalline polymeric blocks having a Tₚ of -5 to 40°C. Such a polymer can be prepared by copolymerizing a mixture of reactants which comprises (i) at least one n-alkyl acrylate or methacrylate in which the n-alkyl group contains at least 12 carbon atoms and (ii) a polysiloxane having a copolymerizable group at one end thereof.

Other polymers which can be used to the coat the microporous film include cis-polybutadiene, poly (4-methylpentene), polydimethyl siloxane, and ethylene-propylene rubber.

The gas-permeable membrane preferably has one or more of the following properties
(i) a P₁₀ ratio, over at least one 10°C range between -5 and 15 °C or between 10 and 20 °C, of at least 2.0 to 2.8;
(ii) an oxygen permeability at all temperatures between 20° and 25°C of 2,480,000 to 7,000,000 ml/m².atm.24 hr. (160,000 to 450,000 cc/100 in².atm.24hr); and
(iii) an R ratio of at least 2.0, preferably at least 3.0, particularly at least 3.5.

The permeability of the container can be influenced by perforating the container in order to make a plurality of pinholes therein.

When using a source of ethylene (in addition to ethylene from ripening bananas themselves), the source of ethylene can make ethylene available immediately after packaging the bananas, or after a desired delay.

Any convenient source of ethylene can be used. I have obtained good results using 2-chloroethyl phosphonic acid, which is often referred to herein as 2CPA. 2CPA can be used in the form of an aqueous solution, for example of concentration 3-4%. The rate at which 2CPA generates ethylene increases with increasing pH of the aqueous solution, which can be adjusted, for example to more than 4, particularly more than 7, by the addition of suitable materials, for example buffer solutions and/or sodium bicarbonate solutions. In one embodiment, a 2CPA solution and a pH adjuster are adsorbed on the same or different absorbent pads, e.g. paper pads, and the pad(s) placed in the bottom of the bag and covered with a polymeric sheet before the bananas are placed in the bag. In another embodiment, a solution of 2CPA is applied to the green bananas, for example by dipping or spraying, before the bananas are placed in the bag.

The invention can in principle be used for any quantity of bananas, for example at least 4 kg, e.g. 16 to 22 kg, of bananas, or smaller quantities, e.g. 1 to 2.5 kg.

### EXAMPLES

The invention is illustrated in the following Examples, a number of which are comparative Examples, designated by the letter C before the number of the example. The bananas, bags and control members used in the Examples were as follows.

### Bananas

The bananas were Cavendish bananas, from Ecuador in Examples 1A-B, C11-12, 2, C2, 4A-B and C41-42, from Costa Rica in Examples 5 A-C and C5, and from Colombia in the other Examples.

### Bags

The large bags were about 0.96 m (38 in.) wide and about 1.2 m (50 in.) long and were made from polyethylene film about 0.056 mm (2.2 mil) thick (available from Roplast Industries under the tradename RA 3030). The polyethylene film had an OTR at 13 °C of about 2915 (188) and at 22 °C of about 4,650 (300), and EtTR at 13 °C of about 11,400 (735) and at 22 °C of about 18,100 (1,170), an R ratio of about 4.5, and a P10 ratio (between 0 and 10 °C.) of about 1.76. The small bags were about 0.3 m (12 in.) wide and about 0.46 m (18 in.) long, and were made from the same polyethylene film.

### Control Members

The Type S control members were as described in copending commonly assigned U.S. Application Serial No. 09/121,082 and corresponding International Publication No. WO 00/04787 and comprised a microporous polyethylene film coated with a polysiloxane/SCC block copolymer. The Type S members had an OTR at 13 °C of about 3,803,850 (245,410) and at 22 °C of about 5,000,000 (324,000), an EtTR at 13 °C of about 16,280,000 (1,050,300) and at 22 °C of about 19,500,000 (1,260,000), an R ratio of about 3.8, and a P10 ratio (between 0 and 10 °C.) of about 1.8. The microporous polyethylene film contained 50-60% silica, had a thickness of about 0.18 mm (0.007 inch), a tear strength of about 90g, a porosity of about 65%, an average pore size of about 0.1 micron and a largest pore size of 4-10 microns (available from PPG industries under the tradename Teslin SP 7). The block copolymer was prepared by the reaction of a polydimethyl siloxane terminated one end only by a methacryloxypropyl group (available from Gelest under the tradename MCR M17), 40 parts, dodecyl acrylate, 26.8 parts and tetradecyl acrylate, 33.2 parts, as described in Example A7 of U.S. Application Serial No. 09/121,082 and corresponding International Publication No. WO 00/04787

The Type A control members were as described in copending commonly assigned U.S. Application Serial No. 08/759,602 and corresponding International Publication No. WO 96/38495, and comprised the same microporous polyethylene film coated with an SCC polymer of dodecyl acrylate, 42 parts, tetradecyl acrylate, 53 parts, and acrylic acid, 5 parts. The Type A members had an OTR at 22 °C of about 1,705,000 (110,000), an R ratio of about 4, and a P10 ratio (between 0 and 10°C.) of about 1.4.

In each Example, the control member was secured to a portion of the bag in which one or more round holes had been cut. The effective area of the control member is about equal to the area of the hole or holes in the portion of the bag to which the control member is attached. However, in Examples 1A-B, C11-12, 2, C2, 3A-D and C31-33, the periphery of the control member was heat sealed to the interior of the bag, thus creating a control member of the kind described in United States Patent No. 6,013,293. In the other Examples, the control member was secured to the exterior of the bag by means of a layer of a pressure sensitive adhesive on the peripheral margin of the control member.

The color stages referred to in the Examples are those accepted by the industry and as shown below.

| Color stage | Description |
|---|---|
| 1 | 95% green |
| 2 | 80% green, 20% slightly yellow |
| 3 | 50% yellow, 50% green |
| 4 | 80% yellow, 20% light green |
| 5 | 95% yellow, with slight green color at stem and blossom end |
| 6 | 100% yellow |
| 7 | 100% yellow with brown sugar spots |

Bananas are preferably at color stage 3.5 to 5 when put on retail sale.

Many of the Examples are summarized in Tables 1-8 below. In the Tables, when more than one result is given for a particular Example, this reflects the fact that more than one test was carried out under the same conditions.

### Examples 1A-B, C11-12, 2 and C2

Each of these Examples uses a large bag. In Examples C 11,1A-B and 2, each bag has one S-type control member placed under two or more holes in the bag. In Example C11, the control member had an area of 1935 mm² (3 in²) and was placed under two holes, each of diameter 20.6 mm (0.81 in.). In Example 1 A, the control member had an area of 6450 mm² (10 in²) and was placed under 6 holes, each of diameter 20.6 mm (0.81 in.). In Examples 1 B and 2, the control member had an area of 12,900 mm² (20 in²) and was placed under 6 holes, each of diameter 28.7 mm (1.13 in). Each bag was packed with about 20 kg (44 lb) of green bananas. The bananas had been harvested at week 11 and maintained at 13-14 °C for about 11 days after harvest before being packed. Except in Examples C12 and C2, excess air was extracted from the bags using a vacuum pump, and the bags were then sealed using tie wraps. In Examples C12 and C2, the bags were left open. The bags were maintained at 13 °C. for an extended time,

Examples 1A, 1B, C11 and C12 being terminated at day 62, and Examples 2 and C2 being terminated at day 40. The results are given in Table 1 below. In Example 2, traces of ethylene (generated by the ripening of the bananas) remained in the test chamber from Example 1 and caused the bananas to ripen more rapidly than in the otherwise substantially identical Example 1 B. This demonstrates the desirability of excluding ethylene when long storage periods are needed (and conversely, the ability to accelerate ripening when desired).

**Table 1**

| | | | | | | | |
|---|---|---|---|---|---|---|---|
| | | Example No. | | | | | |
| | | C11 | 1A | 1B | C12 | 2 | C2 |
| Control member | | yes | yes | yes | no | yes | no |
| Total area of holes In bag under control members (mm²) | | 670 | 2000 | 3880 | - | 3880 | - |
| Color stages | | | | | | | |
| first change at day | | > 62 | 44 | 44 | 12 | 26 | 15 |
| days to change from 3.5 to 4.5 | | - | - | - | - | 4.5 | ***** |
| days to change from 3.5 to 5 | | - | ****** | 11 | 7 | **#** | ***** |
| Weight loss (%) | on day 26 | - | - | - | - | 0.35 | 3.7 |
| | on day 41 | 0.38. | 0.45 | 0.60 | 4.73 | - | - |
| Taste and texture | on day 40 | - | - | - | - | Exct | ◆ |
| | on day 62 | UGH | Exct | Exct | Overripe | - | |
| % O₂ (approximate) | | | | | | | |
| at day 7 | | 5.1 | 11.9 | 13.8 | atm | - | atm |
| at day 8 | | - | - | - | atm | 14.35 | atm |
| at day 47 (after climacteric) | | 5.0 | 0.96 | 2.2 | atm | 2.15 | atm |
| % CO₂ (approximate) | | | | | | | |
| at day 7 | | 5.3 | 3.6 | 3.05 | atm | - | atmta |
| at day 8 | | - | - | - | atm | 3.05 | tm |
| at day 29 (after climacteric) | | - | - | - | atm | 8.0 | atm |
| at day 47 (after climacteric | | 5.3 | 7.9 | 8.4 | atm | - | atm |

| | | | | | | | |
|---|---|---|---|---|---|---|---|
| UGH unripe, green and hard. * the bananas had a color of 4.5 when the test was terminated at day 62 Exct excellent taste and texture # test terminated at this point; extrapolation indicates that time to change from color 3.5 to 5 would be 5.9 days. ◆ Bananas removed on day 26 because they were over-ripe. | | | | | | | |

### Examples 3 and C31-33

Each of these Examples uses a large bag. In Examples C31-33 and 3, each bag has one S-type control member placed under one or more holes in the bag. In Example C31, the control member had an area of 967 mm² (1.5 in²) and was placed under a single hole of diameter 20.6 mm (0.81 in.). In Example C32, the control member had an area of 1935 mm² (3 in²) and was placed under 2 holes, each of diameter 20.6 mm (0.81 in.). In Example C33, the control member had an area of 3225 mm² (5 in²) and was placed under 4 holes, each of diameter 19 mm (0.75 in.). In Example 3, the control member had an area of 12,900 mm² (20 in²) and was placed under 6 holes, each of diameter 25 mm (1 in.). In Example C34, the bag did not have a control member. Each bag was packed with about 18.1 kg (40 lb) of green bananas. The bananas had been harvested at week 13, and maintained at 13-14°C for about 11 days after harvest before being packed. Except in Example C34, excess air was extracted from the bags using a vacuum pump, and then securely tied (the bags were not, however, as completely sealed as in Examples 1 and 2). In Example C34, the bags were left open. The sealed bags were cooled to about 13 °C and shipped to Gulfport, Mississippi, and then to San Francisco, California, maintaining the temperature at about 13 °C. In San Francisco, 36 days after packing, half the bags In each Example were opened, and the other half left intact. All the bags were then exposed to ethylene (500-1000 ppm) in a commercial ripening room for about 24 hours. The bananas in the opened bags ripened rapidly in the expected way; thus by day 43, their color was 6, by day 46 their color was greater than 7, and by day 49, they were overripe. The bags which were still sealed were opened on day 49. The results for the bags opened on day 49 are shown in Table 2 below. These Examples demonstrate that bananas harvested at 13 weeks can be transported in a suitably designed bag, and can be ripened into an excellent product by exposure to ethylene, either through the bag or after opening the bag.

**TABLE 2**

| | | Example No. | | | | |
|---|---|---|---|---|---|---|
| | | C31 | C32 | C33 | 3 | C 34 |
| Control member | | yes | yes | yes | yes | no |
| Total area of hole(s) in bag under control member (mm²) | | 335 | 670. | 1140 | 3040 | - |
| Days to change from color stage 3.5 to color stage 5 | | > 8 | > 8 | > 8 | 5.5 | DDU |
| Taste and texture on day 49 | | SGU | SGU | SGU | Exct | DDU |
| % O₂ (approximate) | at day 23 | 8.6 | 9.8 | 12.7 | 15.5 | |
| | at day 46 | 2.9 | 0.6 | 1.8 | 2.2 | |
| % CO₂ (approximate) | at day 23 | 4.45 | 3.65 | 3.3 | 2.85 | |
| | at day 46 | 13.8 | 11.4 | 5.0 | 9.0 | |

| | | | | | | |
|---|---|---|---|---|---|---|
| SGU soft, green and unpalatable DDU dehydrated, decayed and unpalatable by day 47 (day 11 after exposure to ethylene) Exct excellent taste and texture | | | | | | |

### Examples 4A. 4B, C41 and C42

Each of these Examples uses a.small bag. In Examples 4A-B, each bag has one A-type control member placed over four or five holes In the bag. In Example 4A, the control member had an area of 145 mm² (5.7 in²) and was placed over four holes each of diameter 19 mm (0.75 in.). In Example 4B, the control member had an area of 4516 mm² (7 ln²) and was placed over 5 holes, each of diameter 19 mm (0.75 in.). In Example C41, the control member and the holes under it were as in Example 4A, except that the control member was an uncoated microporous film. In Example C42, the bag was intact except for 200 pinholes each about 0.5 mm (26 gauge) in diameter. Each bag was packed with about 1.35 kg (3 lb) of green bananas which had been maintained at 13-14 °C for about 11 days after harvest Except in Example C42, excess air was extracted from the bags using a vacuum pump, and the bags were then securely tied. In Example C42, the bags were left open. After three days, to allow the packaging atmosphere to equilibrate, the bags were exposed to ethylene (500-1000 ppm) in a ripening room. The results are shown in Table 3 below. These Examples demonstrate that small quantities of bananas can be ripened in a suitably designed bag, and can remain in the bag in excellent condition for several days longer than bananas exposed to the air.

**Table 3**

| | Example No. | | | |
|---|---|---|---|---|
| | 4A | 4B | C41 | C42 |
| Control member | yes | yes | | no |
| Total area of holes in bag over control member (mm²) | 1140 | 1425 | 1140 | - |
| Color stage on day 10 after ethylene treatment | 4.0 | 4.4 | 7.0 | 6.8 |
| Weight loss (%) on day 10 after ethylene treatment | 0.57 | 0.72 | 1.05.. | 0.61 |
| Taste & texture on day 10 after ethylene treatment | Exct | Exct | Overripe | Overripe |

| | | | | |
|---|---|---|---|---|
| uncoated microporous film Exct excellent taste and texture | | | | |

### Examples 5A, 5B, 5C and C5

These Examples show that the bananas generate heat more evenly when ripened in a container including an atmosphere control member. In each Example, a large bag was packed with about 18.1 kg (40 lb.) of green bananas. The green bananas had been harvested 13 days previously and had been stored at 13-14 °C since harvest. A temperature sensor (available from Sensitech, Beverly, Massachusetts, under the tradename Temptale P) was inserted into one banana in each bag. In each of Examples 5A, 5B and 5C, the bag had two S-type control members, each having an area of 11,300 mm² (17.5 in²).Each control member was placed over a single hole in the bag, the hole having an diameter of 70 mm (2.75 in.) in Example 5A, 74.4 mm (2.93 in.) in Example 5B, and 78.7 mm (3.1 in.) in Example 5C. In Example C5, the bag was perforated so that the bananas were surrounded by air. The bags were then sealed with rubber bands. The sealed bags were placed in a refrigerated room at about 13 °C. After about 84 hours, the temperature of the room was raised to about 16.7 °C and after about 12 hours, an ethylene generator was used to provide an initial ethylene concentration in the room of 500-1000 ppm. About 24 hours after the generation of ethylene had begun, the room was vented. The temperature of the bananas was monitored for about 15 days, and reached a peak at about 60 hours after the generation of ethylene had begun. At that time, the concentration of O₂ and CO₂ was measured. The results are shown in Table 4 below. It will be seen that the peak temperature was substantially lower in the bags containing control members than in the perforated bag.

**Table 4**

| | Example No. | | | |
|---|---|---|---|---|
| | 5A | 5B | 5C | C5 |
| Control member | yes | yes | yes | no |
| Total area of holes in bag under control members (mm²) | 7700 | 8700 | 9700 | - |
| Temperature (°C) of bananas 12 hrs after temperature of room was set to 16.7 °C | 16.3 | 15.9 | 15.7 | 16.6 |
| Peak Temperature °C | 21.2 | 21.1 | 20.9 | 23.9 |
| Difference between peak temperature and 16.6 °C | 4.9 | 5.3 | 5.2 | 7.3 |
| % O₂ 60 hours after injection of ethylene | 2.2 | 1.75 | 1.9 | 20.95 |
| % CO₂ 60 hours after injection of ethylene | 7.95 | 6.1 | 7.4 | 0.03 |

### Examples 6 A-E

Each of these Examples uses a large bag having two S-type control members, each control member having an area of 11,300 mm² (17.5 in²). Each control member was placed over seven holes in the bag, each hole of diameter 25.4 mm (1 in). A paper pad about 300 x 400 mm (12 x 16 in.) impregnated with an aqueous solution of 2CPA (3.9%) was placed in the bottom of each bag and covered with a sheet of polyethylene. The amount of the solution varied from Example to Example, and is shown in Table 5 below. About 18.1 kg (40 lb.) of green bananas were then placed in each bag, and the bags were sealed with rubber bands. The green bananas had been maintained at 13-14 °C for about 11 days after harvest. The sealed bags were left in a cold room at 13-14 °C. The color stage of the bananas was monitored, and Table 5 below shows the time in days taken to reach color stages 4 and 5.5.

**Table 5**

| | Example No. | | | | |
|---|---|---|---|---|---|
| | 6A | 6B | 6C | 6D | 6E |
| Control member | yes | yes | yes | yes | yes |
| Total area of holes in bag under control members (mm²) | 7100 | 7100 | 7100 | 7100 | 7100 |
| mL of 3.9% 2CPA solution on paper pad | 30 | 50 | 100 | 200 | 500 |
| Days to color stage 4 | 11 | 10.8 | 10.6 | 11 | 9.6 |
| | * | 20.4 | 20.1 | 12 | 12 |
| | * | 10.5 | 11 | 11 | 11 |
| Days to color stage 5.5 | 17.5 | * | 17.4 | 16 | 16.1 |
| | * | * | 24.2 | 16 | 16.9 |
| | * | 17.5 | 17.4 | 16 | 16.3 |
| Days from color stage 4 to color stage 5.5 | 6.5 | - | 6.8 | 5 | 6.5 |
| | - | - | 3.1 | 4 | 4.9 |
| | - | 7 | 6.4 | 5 | 5.3 |

| | | | | | |
|---|---|---|---|---|---|
| * this color stage had not been reached when the experiment was terminated after 27 days. | | | | | |

### Examples 7 A-D and C71-74

The procedure of Example 6 was followed except for the changes noted below.
1. In Examples 7A-D, there was a single hole, diameter 82.5 mm (3.25 In.), under each of the two control members. The total area of the holes was 10,700 mm².
2. In Examples 7A, 7B and 7C and in comparative Examples C72 and C73, a paper pad impregnated with 0.1 N NaHCO₃ solution was placed adjacent to the paper pad impregnated with 2CPA solution, thus increasing the pH of the 2CPA solution and increasing the rate at which ethylene was generated. The amount of the NaHCO₃ solution varied from Example to Example as shown in Table 6 below.
3. In Examples 7D and C74, 2CPA was not used, but three days after packing, the bags were exposed to ethylene for 24 hours in a conventional ripening room at 16.7 °C and containing 500-1000 ppm of ethylene.
4. Comparative Examples C71-74 were carried out in which no ethylene was used (C71), or the bag was sealed but did not have a control member (C 72-73), or the bag was not sealed (C74).
5. The ethylene concentration in the bags was measured at various times after packing.

The results obtained are shown in Table 6 below.

**Table 6**

| Example No. | 7A | 7B | 7C | 70 | C71 | C72 | C73 | C74 |
|---|---|---|---|---|---|---|---|---|
| Control member | yes | yes | yes | yes | yes | no | no | no |
| mL 3.9% 2CPA solution | 30 | 30 | 30 | no | no | 30 | 30 | no |
| mL 0.1 N NaHCO₃ | 15 | 30 | 60 | no | no | 13 | 30 | no |
| Exposed to ethylene in ripening room | no | no | no. | yes | no | no | no | yes |
| Days to color stage 4 | 12 | 10.2 | 6.2 | 6.5' | | | | 42 |
| | 12.5 | 10.2 | 9.4 | 6.5 | | | | 4.5 |
| | 15 | 8.4 | 9.8. | 7.1 | | | | 4.5 |
| Days to color stage 5.5 | * | * | 9.5 | 11.5 | | | | 6.6 |
| | * | * | 12.5 | 12 | | | | 7 |
| | * | * | 12.9 | 12.3 | | | | 7.2 |
| Days from color stage 4 to color stage 5.5 | - | - | 3.3 | 5 | | | | 2.4 |
| | - | - | 3.1 | 5.5 | | | | 2.5 |
| | - | - | 3.1 | 5.2 | | | | 2.7 |
| Color after 15 days | | | | | 2 | 2 | 2 | |
| ppm ethylene after | | | | | | | | |
| 0 hrs | 0.47 | 4.11 | 8.65 | | | 5.72 | 10.7 | |
| 7 hrs | 0.58 | 2.36 | 10.04 | | | 7.81 | 13.35 | |
| 72 hrs | 0.68 | 1.94 | 6.66 | | | 10.8 | 20.51 | |
| 79 hrs | - | 3.28 | 4.7 | | | 5 | 16.65 | |
| | | | | | | 9.43 | | |
| O₂ after 15 days | 3.73 | 3.97 | 3.72 | | | 0.21 | 0.34 | |
| %CO₂ after 15 days | 6.23 | 6.2 | 4.67 | | | 27.3 | 25.5 | |

| | | | | | | | | |
|---|---|---|---|---|---|---|---|---|
| *this color stage had not been reached when the experiment was terminated. | | | | | | | | |

### Examples 8A-J and C81-83

Examples 8A-J and C 81-83 followed the same procedure as Examples 7A-C and C71-74 except for the changes noted bellow.
1. The ethylene, O₂ and CO₂ concentrations were determined at different times.
2. In some of the examples, the second paper pad was impregnated with 30 mL of an aqueous buffer solution (i) containing potassium phthalate and having a pH of 4, (ii) containing dibasic sodium phosphate, monobasic potassium phosphate, sodium chromate and potassium dichromate, and having a pH of 7, or (iii) containing sodium carbonate and sodium bicarbonate and having a pH of 10. These buffer solutions are available from Orion Research Inc.,Beverley, Massachusetts USA
3. In Examples 8H and C83, the bag was taken to the ripening room 3 days after packing.
4. In Example 8G, the sealed bags were left in a room at about 21 °C (in the other Examples, the room was at 13-14 °C).
5. In Example C83, the bag was not sealed.
The results are shown in Table 7 below.

**Table 7**

| | 8A | 8B | 8C | 8D | 8E | 8F | 8G | 8H | C81 | C82 | C83 |
|---|---|---|---|---|---|---|---|---|---|---|---|
| Control member | yes | yes | yes | yes | yes | yes | yes | yes | yes | no | no |
| mL 3.9% 2CPA solution | 30 | 30 | 30 | 30 | 30 | 30 | 30 | no | no | 30 | no |
| mL 0.1 N NaHCO₃ | no | no | no | 45 | 60 | 75 | 60 | no | no | 60 | no |
| 30 mL of buffer having | pH4 | pH 7 | pH 10 | no | no | no | no | no | no | no | no |
| Exposed to ethylene in ripening room | no | no | no | no | no | no | no | yes | no | no | yes |
| Days to color stage 4 | 11.9 | 15.4 | 13.1 | 9.4 | 8.5 | 9.0 | 82 | 7.7 | * | * | 3.7 |
| | 13.0 | 11.3 | 11.5 | 9.0 | 9.3 | 8.1 | 7.6 | - | - | - | 3.9 |
| | 14.3 | 10:1 | 10.8 | 10. | 8.0 | 8.1 | 6.7 | 10. | - | - | 3.9 |
| | | | | 1 | | | | 6 | | | |
| Days to color stage 5.5 | - | - | - | 15. | 13. | 12. | 14. | 14 | * | * | 5. |
| | - | 15.3 | - | 7 | 8 | 4 | 8 | - | - | * | 6 |
| | - | - | 16.6 | 12. | 13. | 11. | 12. | * | - | - | 6 |
| | | | | 3 | 1 | 4 2 | | | | | |
| | | | | 15 | 11. | 11. | 9.0 | | | | |
| | | | | | 9 | 4 | | | | | |
| Days from color stage 4 to color stage 5.5 | * | * | - | 6.3 | 5.3 | 3.4 | 62 | 6.3 | - | - | 1.3 |
| | * | 4 | - | 3.3 | 3.8 | 3.3 | 4.6 | - | - | - | 2.1 |
| | * | * | 5.8 | 4.9 | 3.9 | 3.3 | 2.3 | - | - | - | 2.1 |
| ppm ethylene after 24 hrs | 0.88 | 1.67 | 1.37 | 3.2 | 4.3 | 5.5 | 10. | 0.4 | 0.3 | 39. | 0 |
| | | | | 5 | 9 | 8 | 9 | 9 | 9 | 5 | |
| %O₂ after 8 days | 3.72 | 5.58 | 2.93 | 3.2 | 2.3 | 2.5 | 1.9 | 2.9 | 17 | 0.3 | - |
| | | | | | 9 | 2 | 5 | 7 | | | |
| %CO₂ after 8 days | 4.73 | 4.7 | 5.3 | 4.9 | 5.1 | 5.4 | 7.9 | 4.7 | 1 | 17. | |
| | | | | 7 | 3 | 7 | 7 | 3 | | 6 | |

| | | | | | | | | | | | |
|---|---|---|---|---|---|---|---|---|---|---|---|
| ^{*} this color stage had not been reached when the experiment was terminated after 17 days. | | | | | | | | | | | |

### Examples 9A-C and C91-92

The procedure of Example 6 was followed, except for the changes noted below.
1. There was a single hole, diameter 82.5 mm (3.25 in.), under each control member. The total area of the hole was 5350 mm².
2. No 2CPA-impregnated paper pad was placed in the bag.
3. The bananas, before being packed into the bag, were dipped into a dilute aqueous solution of 2CPA. The concentration of the 2CPA varied from Example to Example as shown in Table 8 below.
4. Comparative Examples C91 and C92 were carried out in which the bag did not have a control member (C91) or the bananas were not treated with 2CPA solution (C92). Comparative Example C91 is the same as the comparative Examples C71.

The results obtained are shown in Table 8 below.

**Table 8**

| | Example No. | | | |
|---|---|---|---|---|
| | 9A. | 9B | C91 | C92 |
| Control Member | yes | yes | no | yes |
| Concentration of 2CPA (ppm) | 1116 | 128 | 1116 | 0 |
| Days to color stage 4 | 11.9 | 14.6 | * | * |
| | 10 | * | * | * |
| | 11.9 | 11 | * | * |
| Days to color stage 5.5 | * | * | * | * |
| | * | * | * | * |
| | * | * | * | * |

| | | | | |
|---|---|---|---|---|
| * this color stage had not been reached when the experiment was terminated after 27 days | | | | |

Table 9 below shows, for each of the bags in Examples 5A-C, 6A-E and 7A-E, the permeability of the bag to O₂ and to ethylene ("Et" in Table 9), and the respective contributions of the control member and the remainder of the bag. For this calculation, the size of the bag, after sealing, was assumed to be 0.96 x 1.04 m (38 in. x 41 in.), i.e. to have a total area of 2 m² (3115 in²).

**Table 9**

| Example No. | Perm. of bag (mL/atm.24hr) at 13°C | Perm. of bag at 13°C /kg of bananas | Hole area (m² ) | Perm. Of ACM at 13°C | Perm. of rest of bag at 13°C |
|---|---|---|---|---|---|
| C11 | O₂ 8,450 | O₂ 470 | 0.000670 | O₂ 2,550 | O₂ 5,900 |
| | Et 36,000 | Et 2,000 | | Et 10,900 | Et 25,100 |
| 1A | O₂ 13,500 | O₂ 745 | 0.002000 | O₂ 7,600 | O₂ 5,900 |
| | Et 57,650 | Et 3,185 | | Et 32,550 | Et 25,100 |
| 1B | 0, 20.650 | O₂ 1,140 | 0.003880 | O₂ 14,750 | O₂ 5,900 |
| | Et 88,250 | Et 4,875 | | Et 63-130 | Et 25,100 |
| 2 | O₂ 20,650 | O₂ 1,140 | 0.003880 | O₂ 14,750 | O₂ 5,900 |
| | Et 88,250 | Et 4,875 | | Et 63,130 | Et 25,100 |
| C31 | O₂ 7,200 | O₂ 395 | 0.000335 | O₂ 1,300 | O₂ 5,900 |
| | Et 30,650 | Et 1,695 | | Et 5,500 | Et 25,100 |
| C32 | O₂ 8,500 | O₂ 470 | 0.000670 | O₂ 2,550 | 0₂ 5,900 |
| | Et 36,000 | Et 2,000 | | Et 10,900 | Et 25,100 |
| C33 | 0₂ 10,250 | 0₂ 565 | 0.001140 | 0₂ 4,350 | O₂ 5,900 |
| | Et 43,650 | Et 2,400 | | Et 18,550 | Et 25,100 |
| 3 | 0₂ 17,450 | O₂ 965 | 0.003040 | 0₂ 11,550 | O₂ 5,900 |
| | Et 74,600 | Et 4,120 | | Et 49,500 | Et 25,100 |
| 5A | 0₂ 35,000 | O₂ 1,935 | 0.007700 | O₂ 29,100 | O₂ 5,900 |
| | Et 149,800 | Et 8,280 | | Et 124,700 | Et 25,100 |
| 5B | O₂ 39,000 | O₂ 2,155 | 0.008700 | O₂ 33,100 | O₂ 5,900 |
| | Et 166,650 | Et 9,200 | | Et 141,550 | Et 25,100 |
| 5C | O₂ 42,900 | O₂ 2,370 | 0.009700 | O₂ 37,000 | O₂ 5,900 |
| | Et 183,550 | Et 10,150 | | Et 158,450 | Et 25,100 |
| 6 A-E | O₂ 32,840 | O₂ 1,815 | 0.007100 | O₂ 26,940 | O₂ 5,900 |
| | Et 140,500 | Et 7,750 | | Et 115,400 | Et 25,100 |
| 7 A-E | O₂ 46,500 | O₂ 2,570 | 0.010700 | O₂ 40,600 | O₂ 5,900 |
| | Et 199,200 | Et 11,000 | | Et 174,100 | Et 25,100 |

## Claims

1. A package which comprises
(a) a sealed container, the sealed container including at least one atmosphere control member which provides a pathway for O₂, CO₂ and ethylene to enter or leave the packaging atmosphere and which comprises a gas-permeable membrane comprising
(i) a microporous polymeric film, and
(ii) a polymeric coating on the microporous film; and
(b) within the sealed container: bananas and a packaging atmosphere around the bananas;
the sealed container having an O₂ permeability at 13 °C, per kg of bananas in the container (OP13/kg), of at least 700 ml/atm.24 hrs, an R ratio at 13 °C of at least 2; and an ethylene permeability at 13 °C, per kg of bananas in the container (EtOP13/kg) which is at least 2 times the OP13/kg of the container.

2. A package according to claim 1 wherein the sealed container has an OP13/kg of at least 1500 ml/atm.24 hrs.

3. A package according to Claim 1 or 2 wherein the bananas have passed their climacteric, and the packaging atmosphere contains 1.5 to 6% of 0₂, and less than 15%, of CO₂, with the total quantity of 0₂ and CO₂ being less than 16%.

4. A package according to Claim 3 wherein the bananas have passed their climacteric, and the packaging atmosphere contains 1.5 to 3% of O₂, and less than 7%, of CO₂, with the total quantity of O₂ and CO₂ being less than 10 %.

5. A package according to any one of the preceding claims wherein the microporous polymeric film comprises a network of interconnected pores having an average pore size of less than 0.24 micron, with at least 70% of the pores having a pore size of less than 0.24 micron.

6. A package according to any one of the preceding claims wherein the polymeric coating comprises a block copolymer which has a heat of fusion ΔH of at least 5 J/g, and which comprises (i) polysiloxane polymeric blocks, and (ii) side chain crystalline polymeric blocks having a melting point, Tp, of -5 to 40 °C.

7. A package according to any one of claims 1 to 5 wherein the polymer coating on the microporous film is composed of a polydimethyl siloxane.

8. A package according to any one of the preceding claims wherein the sealed container contains at least 15 kg of bananas.

9. A package according to any one of the preceding claims wherein the packaging atmosphere includes ethylene from a ripening room.

## Patentansprüche

1. Verpackung, die
(a) einen versiegelten Behälter, der mindestens ein Atmosphärenkontrollelement einschließt, das einen Weg zur Verfügung stellt, durch den O₂, CO₂ und Ethylen in die Verpackungsatmosphäre eintreten oder diese verlassen können, und das eine gasdurchlässige Membran umfasst, die
(i) eine mikroporöse Polymerfolie und
(ii) eine Polymerbeschichtung auf der mikroporösen Folie umfasst, und
(b) in dem versiegelten Behälter Bananen und eine die Bananen umgebende Verpackungsatmosphäre umfasst,
wobei der versiegelte Behälter eine O₂-Durchlässigkeit bei 13°C pro kg Bananen in dem Behälter (OP 13/kg) von mindestens 700 ml/atm·24h, ein R-Verhältnis bei 13°C von mindestens 2 und eine Ethylendurchlässigkeit bei 13°C pro kg Bananen in dem Behälter (EtOP 13/kg) hat, die mindestens das Doppelte der OP 13/kg des Behälters beträgt.

2. Verpackung nach Anspruch 1, bei der der versiegelte Behälter eine OP 13/kg von mindestens 1500 ml/atm·24h hat.

3. Verpackung nach Anspruch 1 oder 2, bei der die Bananen ihr Klimakterium durchschritten haben und die Verpackungsatmosphäre 1,5 bis 6 % O₂ und weniger als 15 % CO₂ enthält, wobei die Gesamtmenge an O₂ und CO₂ weniger als 16 % beträgt.

4. Verpackung nach Anspruch 3, bei der die Bananen ihr Klimakterium durchschritten haben und die Verpackungsatmosphäre 1,5 bis 3 % O₂ und weniger als 7 % CO₂ enthält, wobei die Gesamtmenge an O₂ und CO₂ weniger als 10 % beträgt.

5. Verpackung nach einem der vorhergehenden Ansprüche, bei der die mikroporöse Polymerfolie ein Netzwerk miteinander verbundener Poren mit einer durchschnittlichen Porengröße von weniger als 0,24 *µ*m aufweist, wobei mindestens 70 % der Poren eine Porengröße von weniger als 0,24 *µ*m haben.

6. Verpackung nach einem der vorhergehenden Ansprüche, bei der die Polymerbeschichtung ein Blockcopolymer mit einer Schmelzwärme ΔH von mindestens 5 J/g umfasst, welches (i) Polysiloxanpolymerblöcke und (ii) kristalline Seitenkettenpolymerblöcke mit einem Schmelzpunkt Tₚ von -5 bis 40°C umfasst.

7. Verpackung nach einem der Ansprüche 1 bis 5, bei der die Polymerbeschichtung auf der mikroporösen Folie aus Polydimethylsiloxan zusammengesetzt ist.

8. Verpackung nach einem der vorhergehenden Ansprüche, bei der der versiegelte Behälter mindestens 15 kg Bananen enthält.

9. Verpackung nach einem der vorhergehenden Ansprüche, bei der die Verpackungsatmosphäre Ethylen aus einem Reifungsraum einschließt.

## Revendications

1. - Emballage qui comprend :
(a) un conteneur scellé, le conteneur scellé comprenant au moins un élément de contrôle d'atmosphère qui fournit un passage pour qu'O₂, CO₂ et l'éthylène pénètrent dans ou quittent l'atmosphère de conditionnement, et qui comprend une membrane perméable aux gaz, comprenant:
(i) un film polymère microporeux ; et
(ii)un revêtement polymère sur le film microporeux ; et
(b) à l'intérieur du conteneur scellé, des bananes et une atmosphère de conditionnement autour des bananes;
le conteneur scellé ayant une perméabilité à O₂ à 13°C, par kg de bananes dans le conteneur (OP13/kg), d'au moins 700 ml/atm.24h ; un rapport R à 13°C d'au moins 2 ; et une perméabilité à l'éthylène à 13°C, par kg de bananes dans le conteneur (EtOP13/kg) qui est d'au moins 2 fois l'OP13/kg du conteneur.

2. - Emballage selon la revendication 1, dans lequel le conteneur scellé a une OP13/kg d'au moins 1500 ml/atm.24h.

3. - Emballage selon l'une des revendications 1 ou 2, dans lequel les bananes ont passé leur climatérique, et l'atmosphère de conditionnement contient 1,5 à 6 d'O₂ et moins de 15 % de CO₂, la quantité totale d'O₂ et de CO₂ étant de moins de 16 %.

4. - Emballage selon la revendication 3, dans lequel les bananes ont passé leur climatérique, et l'atmosphère de conditionnement contient 1,5 à 3% d'O₂ et moins de 7 % de CO₂, la quantité totale d'O₂ et de CO₂ étant de moins de 10 %.

5. - Emballage selon l'une quelconque des revendications précédentes, dans lequel le film polymère microporeux comprend un réseau de pores interconnectés ayant une dimension de pore moyenne de moins de 0,24 micron, avec au moins 70 % des pores ayant une dimension de pore de moins de 0,24 micron.

6. - Emballage selon l'une quelconque des revendications précédentes, dans lequel le revêtement polymère comprend un copolymère à blocs qui a une chaleur de fusion ΔH d'au moins 5 J/g, et qui comprend (i) des blocs polymères de polysiloxane, et (ii) des blocs polymères cristallins à chaîne latérale ayant un point de fusion, Tₚ, de -5 à 40 °C.

7. - Emballage selon l'une quelconque des revendications 1 à 5, dans lequel le revêtement polymère sur le film microporeux est composé d'un polydiméthyl siloxane.

8. - Emballage selon l'une quelconque des revendications précédentes, dans lequel le conteneur scellé contient au moins 15 kg de bananes.

9. - Emballage selon l'une quelconque des revendications précédentes, dans lequel l'atmosphère de conditionnement comprend de l'éthylène provenant d'une salle de maturation.
